

## UNITED STATES PATENT OFFICE

2,026,491

FLANGE OIL AND PROCESS OF MAKING  
SAME

Harry T. Bennett, Tulsa, Okla., assignor to Mid-Continent Petroleum Corporation, Tulsa, Okla., a corporation of Delaware

No Drawing. Application October 10, 1932,  
Serial No. 637,097

4 Claims. (Cl. 196—151)

This invention relates to lubricants and methods of making the same, and more specifically it relates to lubricants for railway track curves and locomotive or car wheel flanges.

- 5 This application is a continuation in part of my copending application, Serial No. 423,558, filed January 25, 1930 relating to lubricants of this kind, which are frequently termed "flange oils".
- 10 Flange oil must adhere or stick tenaciously to metal tracks, or rails, even in the presence of steam, but it must be fluid enough to flow freely from the oiler.

I have found that by distilling the residuum resulting from a fractional distillation of petroleum, an adhesive residuum is produced which has the property of adhering very tenaciously to metal. However, the viscosity of this residual oil, which may range from about 10,000 to 35,000

20 Furol viscosity at 122° F., is so high that said oil cannot be used alone as a flange oil.

I have also found that the product known as pressure tar, which is the residuum produced when petroleum products are cracked while subjected to heat and pressure, has the property of adhering tenaciously to metals. However, the viscosity of this product which may range from 10 to 125 Furol viscosity at 122° F. is too low to be used as a flange oil.

30 I have discovered, however, that an ideal lubricant or flange oil with a Furol viscosity at 122° F. of 200 to 375 can be produced by blending the high viscosity residuum with the pressure tar which has a relatively low viscosity.

35 Usually it requires 50 to 75 percent of pressure tar, and 50 to 25 percent of the high viscosity residuum, to produce an oil which flows as desired. This invention, however, is not limited to the above percentages.

40 In the preferred form of this invention, the high viscosity residuum is obtained by distilling, under a pressure less than atmospheric pressure, a residuum resulting from the fractional distillation of petroleum. The pressure during the distillation operation will usually be from 50 to 200 millimeters absolute pressure.

45 As an example of one form of this invention, I will show how I have made an excellent flange oil as follows:

50 A residuum resulting from the fractional dis-

tillation of petroleum was distilled under an absolute pressure of 60 millimeters until the desired high viscosity residuum was obtained.

This high viscosity residuum was then blended with pressure tar to produce a product with 36 percent of high viscosity residuum and 64 percent pressure tar. An analysis of these two residua is as follows:

|                            | High viscosity<br>residuum | Pressure<br>tar | 10 |
|----------------------------|----------------------------|-----------------|----|
| Gravity                    | 13.1                       | 6.7             |    |
| Sediment (ASTM method)     | 0.2                        | 0.1             |    |
| Furol viscosity at 122° F. | 13,730                     | 50              | 15 |

The blending of the foregoing products produced a flange oil with the following properties:

|                            |     |    |
|----------------------------|-----|----|
| Gravity                    | 8.7 | 20 |
| Furol viscosity at 122° F. | 245 |    |
| Sediment (ASTM method)     | 0.2 |    |
| Flash (Cleveland open)     | 265 |    |
| Fire                       | 365 |    |

As a further illustration of this invention, I have also made an excellent flange oil by blending 31.5 percent of a residuum having a Furol viscosity of 34,668 at 122° F. with 68.5 percent of a pressure tar having a Furol viscosity of 50 at 122° F.

30 The resultant flange oil had the following properties:

|                            |     |    |
|----------------------------|-----|----|
| Gravity                    | 8.0 |    |
| Furol viscosity at 122° F. | 250 |    |
| Sediment (ASTM method)     | 0.2 | 35 |
| Flash (Cleveland open)     | 265 |    |
| Fire                       | 360 |    |

It is understood that this invention is not limited to the foregoing specific examples.

40 I claim:

1. A flange oil having a Furol viscosity between 200 and 375, said oil comprising 50 to 25 percent of an adhesive residuum resulting from a fractional distillation of petroleum and having a Furol viscosity between 10,000 to 35,000 at 122° F., and 50 to 75 percent of an adhesive residuum resulting from a cracking operation and having a Furol viscosity between 10 and 125 at 122° F.

50

2. The process of making flange oils which comprises distilling, under a pressure less than atmospheric pressure, a residuum resulting from fractional distillation of petroleum to provide an adhesive residuum having a Furol viscosity of more than 10,000 at 122° F., and mixing said adhesive residuum with a low viscosity petroleum residuum resulting from a cracking operation and having a Furol viscosity from 10 to 125 at 122° F. to produce a flange oil having a Furol viscosity of more than 200 at 122° F.
3. The process of making flange oils which comprises distilling under a pressure less than atmospheric pressure, a residuum resulting from fractional distillation of petroleum to provide an adhesive residuum having a Furol viscosity of more than 10,000 at 122° F., and mixing with said

adhesive residuum a quantity of a pressure tar resulting from a cracking operation amounting to 50 to 75 percent of the volume of the resultant mixture and having a Furol viscosity from 10 to 125 at 122° F.

4. The process of making flange oils which comprises distilling, under an absolute pressure of 50 to 200 millimeters, a residuum resulting from fractional distillation of petroleum to provide an adhesive residuum having a Furol viscosity be- 10 tween 10,000 and 35,000 at 122° F. and mixing said adhesive residuum with 50 to 75 percent of a petroleum residuum resulting from a crack- 15 ing operation and having a Furol viscosity be- 15 tween 10 and 125 at 122° F.

HARRY T. BENNETT.